

Oct. 19, 1943.

A. E. CALKINS

2,332,202

LUBRICATING GREASE MANUFACTURE AND APPARATUS THEREFOR

Filed Aug. 19, 1941



FIG. - I



FIG. - II

Austin E. Calkins Inventor  
By P. L. Young Attorney

## UNITED STATES PATENT OFFICE

2,332,202

## LUBRICATING GREASE MANUFACTURE AND APPARATUS THEREFOR

Austin E. Calkins, Westfield, N. J., assignor to Standard Oil Development Company, a corporation of Delaware

Application August 19, 1941, Serial No. 407,406

15 Claims. (Cl. 252—39)

This invention relates to a novel process for manufacturing lubricating greases and for apparatus to be used for such processes; more particularly it relates to an improved process which is more convenient and economical than those of the prior art, and especially adapted for the manufacture of lime soap greases.

Heretofore mineral lubricating greases have usually been made in large kettles, either steam heated or directly fired and adapted for open cooking, or cooking under pressure a mixture of saponifiable material, such as animal fat, and a saponifying agent, with or without small additions of water and/or mineral oil. Such cookers having sufficient capacity to handle all the grease required to be manufactured are very expensive and require a large amount of space.

One object of the present invention is to provide a grease manufacturing equipment which avoids the use of large cooking kettles; another object is to accomplish a grease manufacture in equipment which requires much less plant floor space than processes used heretofore; and another object is to provide a process and apparatus which can be operated economically and efficiently and which can be readily adapted to produce the various types and grades of lubricating greases required for the market. Another object is to provide an apparatus which involves far simpler and smaller moving parts than a pressure kettle.

Broadly, the invention comprises making a lubricating grease soap stock by mixing a saponifiable material and a saponifying agent (with or without small additions of other materials, such as water, mineral oil, etc.) in a large, unheated mixing zone, heating small portions of the resultant mixture outside of the mixing zone, and recycling the same to the mixing zone until the entire mixture has been substantially completely saponified by use of a plurality of mixing zones, one or more of which can be used for mixing while the soap stock from another is being discharged either into storage or into suitable grease-blending equipment. The invention is particularly adapted for preparing a continuous supply of soap stock which in turn is intended to be continuously and directly fed into a continuous grease-blending unit continuously compounding controlled proportions of the soap stock and mineral oil, which continuous blending is claimed in copending application 342,081 filed June 24, 1940, of which the present application is a continuation-in-part, thus providing a simple and efficient process and apparatus for the continuous manufacture of lubricating greases which have heretofore been made by batch processes.

The invention will be better understood from a description of the accompanying drawing in

which Fig. I illustrates in a schematic layout one embodiment of the invention, and Fig. II shows an alternative method of charging a mixing zone, although it is not intended that the invention be limited to the particular type of equipment used, where other equipment, somewhat different in shape, for instance, would accomplish the same or substantially equivalent purposes.

As indicated in the drawing, one or more mixing tanks 1 (two are shown in Fig. I) are provided for mixing the materials to be used in making a concentrated soap stock. These materials may either be fed in at the top by opening or removing the lid, or, as shown in Fig. II, may be fed in through suitable inlet feed lines, i. e., the fat or other saponifiable material through line 2, represented as a screw conveyor feed, the lime and water being suitably fed in as a slurry through line 3, and the mineral oil, if desired, through line 4, or these various materials may be measured in separate vessels and pumped in through line 23 as will be explained later. The mixer 1 is provided with an outlet suitably located, such as part-way up one side, for pumping the saponification mixture through line 5 by means of pump 6 into heater 7, which may be of any convenient type, but preferably consists of a steam-heated pipe coil. In this heater, the portion of saponification mixture being fed through line 5 is raised to a temperature at least as high as saponification temperature, e. g., between the approximate limits of 250°—550° F., or for a lime soap stock, preferably between the approximate limits of 300° F. and 400° F., and the saponification mixture, which is at least partially saponified by the thus described heating, is recycled by line 8 back to the bottom of the mixer 1.

An important feature of the invention is that the pump 6 which may suitably be a high capacity gear pump should have a high capacity relative to the volume of the mixer 1 and should be able, for instance, to circulate a volume of material equal to the volume of the mixer in less than 2 or 3 minutes. The heating and recycling is continued until the entire mixture of materials is substantially completely saponified, at which time the valves at the bottom of the mixing tank 1 are reversed, i. e., by closing the valve on the recycling line 8 and opening the discharge valve in line 10, from which the saponified mixture is now withdrawn as a finished soap stock which may be either passed to storage with or without going through the cooler 11, or if desired, passed on through line 12 to a suitable grease-mixing equipment. This latter may be designed for batch operation in conventional kettles or, preferably, continuous as shown in the drawing, namely, by passing the soap stock from line 12 through a metering soap pump 13 to a high-speed mechanical mixer 14, such as a

Lancaster disperser, into which mineral oil of suitable viscosity from a suitable source (not shown) is fed through line 18, oil heater 16, line 17, and metering oil pump 18. The finished lubricating grease is discharged from the mixer 14 through line 19 and, if desired, through a filter 20 and a pressure control valve 21 and finally through outlet 22. By-pass line 24 is used if it is desired to feed raw material into mixers 1 by means of line 23.

Connections should be made to the mixing tanks, circulating pumps, heater, and various lines through which fat or soap stock must pass, so that they may be blown clear of soap ingredients before being allowed to cool. A plurality of mixing tanks may be so connected that while one is being discharged through the cooler into the grease-mixing equipment, one or more other mixing tanks are being used for mixing and heating other batches of soap stock, with the result that a substantially continuous supply of soap stock is maintained for feeding to the grease-mixing equipment. If more than two mixing tanks are to be used for mixing at the same time, one or more additional heaters and circulating pumps may be used.

If desired, an auxiliary heater or cooker may be provided in line 100 in order to give the soap stock being discharged from the mixing tank a final heating before going to the grease-mixing equipment, with or without the use of the cooler 11.

Instead of using steam for heating the heater 7, one may use higher boiling heating media, such as diphenyl oxide (boiling point 288° C.) which, when vaporized like steam, permits the use of temperatures up to 750° F. or so, as for use with sodium soap which requires about 450° F. for good fluidity, or mixed heating media, such as mixtures of diphenyl oxide and diphenyl, mercury, etc., or high temperature liquid heating media, such as molten salts, or hot gases, such as flue gas or other combustion gases, or direct firing may be used, if desired, although steam is preferred for temperatures below 350° F. because it is cheapest and adapted to efficient and accurate control of the temperature and leads to the production of uniform quality in the soap stock.

If desired, an auxiliary pump may be used to assist in discharging the soap stock from the mixing tanks through line 10, or these tanks may be discharged by building up a pressure in the top of the tank by steam or other fluid pressure.

A condenser 25 may be provided in order to condense steam which may be drawn off from the top of the mixing tank 1 and also, if desired, to recover glycerine vapors.

Suitable shut-off valves, thermometers, thermostats, safety valves, and pressure control valves are provided in order to carry out the invention as described; preferably, the equipment is designed for continuous, automatic operation for the manufacture of the soap stock, and this, in turn, is combined preferably with a continuous and automatic grease-blending operation.

The cooler 11 may be of any suitable construction, such as a straight section of pipe, or one or more coils of pipe passing through a water- or oil-cooling jacket or shell, or preferably of the scraped screw type.

If an auxiliary heater is used in line 10, the rate of feed therethrough should be regulated with the time (according to the length of internal pipe) so that there will be a constant flow of soap stock to the grease mixer, if desired.

As an example of the use of the above-described equipment, it may be mentioned that if a calcium soap stock is to be made from a mixture of hog fat and hydrated lime, based on 20% fatty acid, a temperature of about 250° F. is required to insure a fluid condition at all times in order to obtain a substantially homogeneous mixture, and in order to insure complete saponification, the temperature is preferably raised somewhat higher, e. g., between about 300° and 400° F., this being accomplished either entirely in the heater 7, or partly therein and partly in a slurry heater (not shown) in line 10, as suggested above. If desired, the fat may be pre-heated in a heater (not shown) ahead of line 2.

Operation of a soap-manufacturing unit, such as described above, has demonstrated that the time required to prepare one mixer volume of satisfactory grease soap stock is less than 1 hour, compared to at least 3½ or 4 hours heretofore required with the customary pressure-kettle operation. Large savings in equipment cost are also realized. Operation of a unit according to this invention indicates, for instance, that a manufacturing plant no larger than 6 x 6 x 13 feet using three mixing tanks consisting of round pipes 6 feet high, 20 inches in diameter, and truncated at the bottom, has sufficient capacity for producing about 6,000,000 to 8,000,000 pounds of lubricating grease per year.

As indicated in the drawing, the mixing tank 1 preferably consists of a vertical pipe with a truncated bottom, because this type of mixer obtains suitable mixing of the ingredients by the mere pumping off through an outlet part-way up the side and recycling the heated materials back into the mixer at the bottom; if desired, baffle plates may be used to assist in obtaining desired mixing. Also, if desired, mechanical mixing, as with a motor-driven stirring arm or blade, may be used, although normally this is not necessary. Various other types of mixing zones may be used as, for instance, an almost horizontal, rotary drum adapted to be fed in slowly at the higher end and to be slowly and continuously discharged at the lower end. Such a drum may be provided with baffle plates to assist in mixing the ingredients or with a stationary or rotary mechanical mixing arm. The large capacity screw conveyor can also be used as the mixing zone, the materials being fed in at one end and discharged continuously at the other end, although in this case provision would have to be made to reverse the direction of the screw conveyor after the recycling is finished in order to draw off the soap stock into the grease-blending equipment, or else provide an outlet between the screw conveyor and the heater for drawing off the finished soap stock.

The saponifiable material to be used may be any of the fats, fatty oils, fatty acids, etc., commonly used for making lubricating grease. Specific examples of such materials include beef stearin, mutton tallow, hog fat, oleic acid, stearic acid, tallow fatty acids, lard oil, soya bean oil, cottonseed oil, corn oil, neats-foot oil, and similar animal and vegetable oils, hydrogenated fatty oils, such as hydrogenated fish oils, or synthetic fats and acids, such as wax oxidation acids, etc. Of these various types of materials, hog fat, degras, lard oil, tallow, oleic acid, and other fatty acids are preferred, especially for making lime soap greases.

As the saponifying agent, lime is preferred and this may be used either in the form of calcium

hydroxide or calcium oxide, although the former is preferred. Other alkaline earth metal bases may be used, such as gelatinous magnesium hydroxide or magnesium oxide, and corresponding barium or strontium compounds. Although the invention is particularly applicable to the preparation of alkaline earth metal soap greases, other saponifying agents may be used, such as caustic soda, caustic potash, lithium hydroxide, gelatinous aluminum hydroxide, etc. If desired, alkali metal soaps may be converted into corresponding aluminum soaps, as by treating with aluminum sulfates. Also, mixtures of several different saponifying agents may be used, such as, lime and soda, lime and potash, soda and barium, lime and barium, etc.; in such mixtures the saponifying agent from group II-A of the Mendeleeff Periodic Table should preferably be at least 90% of the total base.

As indicated earlier, it is desirable with certain types of greases, particularly the lime greases, to have a small amount of water present in order to obtain the best grease structure and the optimum yield, expressed in volume of grease produced for any particular soap content. For lime soap greases, it is preferable to have a water content of approximately .05 to .15% of water for each percent of lime soap present. For other than lime soap greases considerably less water should be present, for instance, in a soda soap grease the maximum water content should be about 1%, i. e., soda soap greases are usually substantially dehydrated; and in the case of aluminum soap greases generally the water content should be 0 or as near thereto as is practicable. If the saponifiable material used is a glyceride or a mixture of glycerides, some glycerine is formed as a by-product of the saponification reaction, and whatever water is desired in the finished grease must be added, and, in fact, generally a slight excess of water must be added initially, in order to compensate for the small amount of water which is lost by vaporization during the preparation of the soap stock and final grease blending. On the other hand, if fatty acids are used as the saponifiable material, then some water is formed as by-product during the saponification, and in such a case little, if any, additional water need be added.

As referred to earlier, it is possible to make various soap stocks without having any mineral oil present, but it is preferred to prepare the soap stock in the presence of a small amount of mineral oil, usually less than 30% of the weight of saponifiable material, and preferably about 10-20% of the weight of saponifiable material. The mineral oil for this purpose may be of any particular type, as to whether it is paraffinic, naphthenic, or mixed base oil, although paraffinic is usually preferred, and of the particular boiling range and viscosity range intended to be used in the finished grease composition; or, since only a relatively small amount of the oil is used in making the concentrated soap stock, a mineral lubricating oil of widely varying boiling range and viscosity may be used for this purpose, as one example, an oil having a relatively pale color and a Saybolt viscosity between the approximate limits of 40 seconds and 60 seconds at 210° F., this concentrated soap stock then being blended with a much larger proportion of a mineral oil of the desired characteristics for making the finished lubricating grease.

As a general guide for the preparation of concentrated soap stocks according to this invention

and the subsequent blending of the latter with mineral oil to form the finished lubricating greases, the following table is given to show the approximate range of proportions of materials to be used (expressed in percent by weight). Since the amounts required, or at least preferred for best operation, differ according to the type of base or saponifying agent used, proportions are given for soap stocks made from three different bases, namely, calcium, sodium, and aluminum.

Table

|         | Concentrated soap stock |                  |                |            | Finished<br>grease<br>Soap |
|---------|-------------------------|------------------|----------------|------------|----------------------------|
|         | Oil                     | H <sub>2</sub> O | Soap           | Glyc.      |                            |
| Ca..... | 0-50<br>35-70           | 3-12<br>0-1      | 45-80<br>30-75 | 0-8<br>0-8 | 1-35<br>1-35               |
| Na..... | 50-85                   | 0                | 15-50          | 0-5        | 1-15                       |
| Al..... |                         |                  |                |            |                            |

In the table, the portion dealing with the concentrated soap stock shows not only the proportion of soap but also the use of water and glycerine in some instances and indicates that some oil is always used, because operations (especially the final grease-blending) are substantially facilitated when some mineral oil is present in the preparation of the soap stock, although, as explained previously, it is possible to make the soap stock without any mineral oil. In the portion of the above table pertaining to the finished grease composition, only the figures are given for the soap content, because greases are usually blended from controlled amounts of soap stock and mineral oil in order to obtain a grease of some particular soap content as required by the purchaser's specifications; the amounts of mineral oil, water, and glycerine in the finished grease can readily be calculated from the amounts of those constituents in the soap stock and the proportion of mineral oil blended with the soap stock.

Although the invention is particularly adapted to the preparation of concentrated soap stock to be subsequently blended with a large proportion of mineral oil to make a finished grease, it is also possible to use the same equipment for directly producing a finished lubricating grease, by merely using the correct final amount of mineral oil in the original mixture. Ordinarily, however, this procedure is not preferred because the large amount of mineral oil present dilutes the saponification mixture, and, therefore, usually requires a somewhat higher temperature or longer time to insure complete saponification, and also because from a practical plant operation point of view, it is usually suitable and more convenient to make the various grades of lubricating grease having different penetration and viscosity characteristics by making a large batch of concentrated soap stock and blending portions thereof with various amounts of mineral oil, rather than making up separate batches of soap stock for each grade of grease.

For the sake of illustration, the following specific examples are given:

## Example 1

|                     | Pounds parts |
|---------------------|--------------|
| Hog fat .....       | 306.0        |
| Hydrated lime ..... | 43.1         |
| Caustic soda.....   | 1.5          |
| Water.....          | 29.0         |
| Mineral oil.....    | 89.0         |

70 were charged to the tank and circulation started

through a heater of 19.0 sq. ft. inside surface with 115 lb. per sq. in. steam outside. In 40 minutes the temperature had risen to 321° F., and the soap concentrate was discharged to an open kettle. It was 99.5% saponified, which is much better than the usual 95-98% achieved in 2 hours pressure kettle cooking. The concentrate was blended with oil to give the usual production of lime grease.

*Example 2*

|              | Parts |
|--------------|-------|
| Tallow       | 1000  |
| Tallow acids | 1000  |
| Caustic soda | 290   |
| Water        | 290   |
| Mineral oil  | 2000  |

were charged to the tank and circulation started. The heater steam was at 80 lb. per sq. in. In one hour the temperature was 285° F. Steam was vented from a pressure of 45 lb. per sq. in. to atmospheric pressure in the course of another hour, leaving a substantially dehydrated mass of excellent soda soap grease base.

It is not intended that this invention be limited to the specific examples recited, nor to the particular types of equipment shown in the accompanying drawing which are given merely for illustration, but only by the appended claims in which it is intended to claim all novelty inherent in the invention.

*I claim:*

1. The process of making lubricating materials which comprises mixing a saponifiable material, a saponifying agent and a small amount of mineral oil, heating relatively small portions of the resultant mixture outside of the mixing zone to a temperature at least as high as the saponification temperature, and recycling the same continuously to said mixing zone until the entire mixture is saponified.

2. Process according to claim 1 in which the mixing and recycling are effected by means of a pump having a sufficiently high capacity to circulate a volume of material equal to the volume of the mixing zone in a period of less than 3 minutes.

3. The process of making a calcium soap stock for manufacturing lubricating greases which comprises mixing a saponifiable material, a calcium saponifying agent and a small amount of mineral oil in a mixing zone, heating small portions of the resultant mixture outside of said mixing zone in a pipe-coil heater to a temperature at least as high as saponification temperature, and continuously recycling the said mixture to the mixing zone until the entire mixture is substantially completely saponified, said mixing, heating, and recycling being carried out in a closed system under a superatmospheric pressure.

4. A process according to claim 3 in which animal fat and hydrated lime are used and the saponification mixture is heated to about 300°-400° F.

5. The process of making a calcium soap stock having approximately the following composition, in percent by weight:

| Material:    | Per cent |
|--------------|----------|
| Calcium soap | 45-70    |
| Water        | 5-12     |
| Glycerine    | 0-8      |
| Mineral oil  | 10-50    |

for use in preparation of lubricating greases, which comprises mixing animal fat, hydrated lime, and mineral oil in proportions required to 75

produce a soap stock having the above composition, in an unheated mixing tank, continuously withdrawing small portions of the resultant saponification mixture and heating same outside of the mixing tank in a steam-heated pipe coil to impart thereto a temperature of about 300°-400° F., and continuously recycling said heated portions to the mixing zone until the entire mixture is substantially completely saponified, and then discharging the finished calcium soap stock from the mixing tank.

6. The process of making a lubricating grease soap stock which comprises mixing a saponifiable material, a saponifying agent, and a small amount of mineral oil in an unheated mixing zone, continuously heating small portions of the resultant mixture outside of the mixing zone in a steam-heated pipe coil to a temperature at least as high as saponification temperature, and continuously recycling said heated portions to the mixing zone until the entire mixture is substantially completely saponified, and finally stopping the circulation through the heater and discharging the finished soap stock through a cooler.

7. The continuous process of making a lubricating grease soap stock which comprises mixing a saponifiable material, a saponifying agent, and a small amount of mineral oil alternately in a plurality of unheated mixers, withdrawing small portions of the resultant mixture from at least one of said mixers, heating said small portions outside of the mixer to a temperature at least as high as saponification temperature, and recycling said heated portions to the mixer from which they were withdrawn, repeating said withdrawing, heating, and recycling until the mixture is substantially completely saponified, then starting a similar mixing, heating, and recycling in at least one other mixing zone, and gradually discharging the soap stock from the first mixing zone at such a rate that said zone will become substantially empty at about the time when the saponification of the second mixing zone is substantially complete, thus coordinating the rate of saponification and discharging that a substantially continuous flow of finished soap stock is produced.

8. Process according to claim 7 in which the mixing, heating, and recycling to any one mixing zone is stopped after the mixture has been heated sufficiently to effect partial saponification but stopped before the saponification has been completed, and then the mixture being finally discharged from the mixing zone is passed through an auxiliary heater wherein the saponification is completed and the finished soap stock is discharged at the desired temperature.

9. The continuous process of making a lubricating grease which comprises mixing a saponifiable material, a saponifying agent, and a small amount of mineral oil alternately in a plurality of unheated mixers, withdrawing small portions of the resultant mixture from at least one of said mixers, heating said small portions outside of the mixer to a temperature at least as high as saponification temperature, and recycling said heated portions to the mixer from which they were withdrawn, repeating said withdrawing, heating, and recycling until the mixture is substantially completely saponified, then starting a similar mixing, heating, and recycling in at least one other mixing zone, and gradually discharging the finished soap stock from the first mixing zone at such a rate that said zone will become substantially empty at about the time when the sa-

ponification of the second mixing zone is substantially complete, thus coordinating the rate of saponification and discharging that a substantially continuous flow of finished soap stock is produced, and continuously blending the resultant soap stock in controlled proportions with heated mineral oil to produce a finished lubricating grease.

10. The continuous process of making a calcium base lubricating grease which comprises continuously making a calcium soap stock having approximately the following composition, in percent by weight:

| Material:    | Per cent |
|--------------|----------|
| Calcium soap | 45-70    |
| Water        | 5-12     |
| Glycerine    | 0-8      |
| Mineral oil  | 10-50    |

by mixing animal fat, hydrated lime, and a small amount of mineral oil in proportions required to produce a soap stock having the above composition, in a plurality of mixing zones, withdrawing small portions of the resultant mixture from at least one of said zones, heating said small portions outside of the zone to a temperature at least as high as saponification temperature, and recycling said heated portions to the zone from which they were withdrawn, repeating said withdrawing, heating, and recycling in at least one other mixing zone, and gradually discharging the calcium soap stock from the first mixing zone at such a rate that said zone will become substantially empty at about the time when the saponification of the second mixing zone is substantially complete, thus coordinating the rate of saponification and discharging that a substantially continuous flow of finished calcium soap stock is produced, and continuously blending the resultant calcium soap stock in controlled proportions with heated mineral oil to produce a finished lubricating grease.

11. The process of making a lubricating grease which comprises mixing a saponifiable material and a saponifying agent in proportions to produce a lubricating grease soap stock, in an unheated mixing zone, continuously withdrawing small portions of the resultant mixture and heating said small portions outside of the mixer to a temperature at least as high as saponification temperature, recycling said heated portions to said

5 mixing zone, and repeating said withdrawing, heating, and recycling until the entire mixture is substantially completely saponified, discharging the finished soap stock from said mixing zone through a temperature regulator to impart to the soap stock the temperature required for grease-blending, and blending the resultant soap stock in controlled proportions with heated mineral oil to produce a finished lubricating grease.

10 12. The process of making a soda base grease soap stock which comprises mixing a saponifiable material, caustic soda and a small amount of mineral oil, heating relatively small portions of the resultant mixture outside of the mixing zone to a temperature at least as high as the saponification temperature and recycling same continuously to said mixing zone until the entire mixture is saponified, and substantially completely dehydrating the resultant soap stock.

15 20 13. Apparatus for manufacturing lubricating grease which comprises at least one unheated mixer, means for feeding soap-making materials thereinto, a heating zone outside said mixer, means for continuously circulating small portions of material from the mixer through the heater and for recycling them into a different part of said mixer, and means for blending the resultant soap stock with mineral oil.

25 30 14. Apparatus for the continuous manufacture of a lubricating grease which comprises a plurality of mixers connected so as to be used alternately, means for feeding soap-making materials into feed mixers, a heating zone outside of said mixers, a pump for circulating small portions of material from any one of the mixers through the heater and recycling same into the mixer, means for discharging finished soap stock from said mixers to a continuous grease-blending equipment comprising a high-speed grease mixer, means for continuously feeding controlled amounts of soap stock and heated mineral oil stock into the grease mixer, and means for continuously withdrawing the resultant grease through a cooler.

35 40 45 15. An apparatus according to claim 14 in which the mixers consist of substantially vertical pipes truncated at the bottom, adapted to be charged at the top, pumped out through an outlet located part-way up the side for heating, and adapted to be recycled into the mixer at the bottom.

AUSTIN E. CALKINS.